

## UNITED STATES PATENT OFFICE

2,614,991

## STEAM ENGINE LUBRICANTS

Jones I. Wasson, Union, N. J., assignor to Standard Oil Development Company, a corporation of Delaware

No Drawing. Application March 30, 1950,  
Serial No. 152,979

1 Claim. (Cl. 252—56)

**1**  
The present invention relates to steam cylinder lubricating oil compositions and related products and also to a process of preparing such compositions. More specifically, the invention pertains to an oil composition having the properties of high temperature stability, relative non-volatility, appropriate emulsification, and other qualities which are desirable for the effective lubrication of the cylinders and valves of locomotives or other steam engines and for other and related applications and uses.

In the prior art, it has long been considered necessary to use high grade essentially paraffinic oils for the lubrication of the cylinders and valves of steam engines. These, of course, are relatively expensive. In addition, in order to secure a desired emulsification of the oil so as to coat the wet contacting surfaces adequately, it has been considered necessary to use a substantial quantity of some natural fatty material such as 5 tallow, or the like. Oils which have a tendency to emulsify with condensed steam are considered essential. They should have a high degree of stability at temperatures as high as about 750° F. In the prior art, for example, as in the patent to Lazar, No. 2,084,532, it has been suggested that other materials be used in lieu of the fat, tallow, or the like, which is not only costly but tends to decompose at the high operating temperatures. This patent suggests that a small amount of a lime or magnesium soap may be added to improve the effectiveness of the mineral oil and to reduce substantially the requirements for fatty oil. It also suggests that oils of heavy asphaltic base or of mixed base, suitably refined, may be used in lieu of or with Pennsylvania oil and that residual oils of the Pennsylvania type which contain certain organic acids may be converted by the addition of traces of oxides (which form soaps) into additive products giving the desired emulsification properties.

As also indicated in the aforesaid patent, and as is common knowledge in the prior art, the stability of the steam cylinder oil itself at the high operating temperatures involved is an important consideration. In general, unsaturated oils have been considered unsatisfactory and this is another reason that the relatively expensive straight paraffinic oils, especially the Pennsylvania oils, have been preferred.

The present invention is based upon the discovery that by combining certain specific resinous products which may be derived from Pennsylvania oils, with oils of suitable grade derived from non-paraffinic or predominantly non-par-

affinic bases, an improved lubricant may be prepared which is relatively inexpensive and which is superior in many respects to any of the products of the prior art. Specifically, it has been found that certain resinous materials, which are known to be precipitated from paraffin base or from Pennsylvania oils by treatment with propane, may be combined with the non-paraffinic oils of appropriate viscosity and with a relatively much smaller proportion of tallow than previously used to form an excellent steam cylinder lubricant.

As is well-known in the prior art, paraffinic oils, especially Pennsylvania crude oils, which have their lighter fractions removed, may be dissolved in an excess of liquid propane or other very light hydrocarbons under pressure at ordinary temperatures. The prior art practice is to use at first about two volumes of liquid propane for each volume of Pennsylvania reduced crude, the solution thereafter being cooled by permitting some of the propane to evaporate. Such cooling may cause a separation of some of the wax in the oil and this wax may be removed. 15 Upon addition of further propane up to about 10 volumes per volume of oil and mild heating under pressure, a viscous resinous product of relatively low volatility and high molecular weight is precipitated in the form of a heavy oil to plastic solid material having a viscosity in excess of about 1000 S. S. U. at 210° F. This resinous product per se is well-known in the prior art. It is essentially neutral, being substantially free from acids, though its precise composition is not 20 fully understood. It has been used previously in certain mineral oils of low viscosity (for example, about 150 S. S. U. at 100° F.) as a metal quenching oil, as described for instance in the patent to Rodman No. 1,818,431.

25 The present invention uses the same resinous propane precipitated residue as a modifier for the non-paraffinic oil. It should be employed in proportions of about 3 or 4 to 12% by weight, based on the total composition, in predominantly non-paraffinic oils, for example, a Mid-Continent oil of about 135 to 300 S. S. U. viscosity at 210° F. It is preferred to add to such combined ingredients from about 2 to about 5% of fatty oil, preferably tallow. It will be noted that the 30 principal ingredient is the relatively inexpensive lubricating oil of non-paraffinic base in proportions of 83 to 94% by weight.

A specific composition which has been found to be very satisfactory consists of about 87% by 35 weight of a Mid-Continent or predominantly non-

paraffinic base oil of about 210 S. S. U. viscosity at 210° F., containing about 10% of the viscous resinous material described above which has a viscosity of over 1,000 S. S. U. at 210° F., and about 3% of tallow or other animal fat. It is emphasized that the resulting product is a high grade steam cylinder oil which has a viscosity of between 4,000 and 5,000 S. S. U. at 100° F. Other inspections are as follows: flash 595° F., viscosity at 210° F. 230 S. S. U., viscosity index 93, Conradson carbon 4.3% and ASTM pour point +25° F.

Another composition which is moderately successful consists of 93% of the oil of non-paraffinic origin, 4% of the viscous propane precipitated resin from Pennsylvania oils and 3% of tallow.

Both of the products just described were tested in large two-cylinder and four-cylinder Baldwin steam locomotives operating at steam pressures of 220 to 235 p. s. i. and steam temperatures of 600° to 700° F., the tractive effort being 63,200 to 115,000 pounds. The locomotives were operated on the lubricants in passenger car service and also under very severe conditions in freight service in a mountainous region. As controls, a cylinder oil containing 97% of the Mid-Continent oil and 3% of tallow, and a cylinder oil containing 97% of a Pennsylvania oil and 3% of tallow, were also tested. The results of the tests under severe conditions in freight service are shown in the table below:

*Steam locomotive tests*

| Cylinder Oil                                                     | Lubrication Results        |
|------------------------------------------------------------------|----------------------------|
| Mid-Continent Oil of 210 S. S. U. at 210° F.:<br>+3% Tallow----- | Poor, Rods Dry and Bluish. |
| +3% Tallow +4% Resin Fraction-----                               | Excellent.                 |
| +3% Tallow +10% Resin Fraction-----                              | Do.                        |
| Pennsylvania Oil: +3% Tallow-----                                | Do.                        |

The Mid-Continent oil containing only tallow gave very unsatisfactory results, the cylinder rods being dry and bluish indicating inadequate lubrication. Similar results (not shown in the table) were obtained when the Mid-Continent oil was topped to a viscosity of 300 S. S. U. at 210° F. prior to blending with 3% tallow, showing that increasing the concentration of heavy fractions of Mid-Continent oil in this manner has no beneficial effect. On the other hand, the compositions of this invention containing as little as 4% or as much as 10% of the resin fraction were just as satisfactory as the cylinder oil blend containing the straight Pennsylvania oil, giving excellent lubrication of the locomotives in heavy duty service. The Mid-Continent base oil containing 10% of the resin fraction and 3% tallow has been continued in this service as a service test for a number of months, with particularly satisfactory results.

It is also emphasized that the resinous fractions obtained by propane precipitation from Pennsylvania residual oils which are used as additives to Mid-Continent oils are very viscous heavy products which must be used in controlled proportions within about the limits specified above (3 to 12%, preferably 4 to 10% by weight of the total com-

position) to obtain satisfactory products. Products which perform fairly well may be obtained by combining the resin with the oil, omitting the fatty material altogether. Products containing both the propane extracted resins and also fats, such as tallow, in proportions of 2 to 5%, especially about 3%, give a very superior performance. With such compositions, it is not necessary to use soap of any kind, which is highly advantageous. Soaps leave residues which are frequently objectionable.

While the reasons for superior performance of the composition of this invention are not entirely clear, it is believed that the resins extracted from paraffinic type residual oils form a relatively non-fugitive lubricating film on the relatively moving metal surfaces, even at the high temperatures involved. Since these resinous materials appear to be essentially neutral and are apparently quite fully saturated, they do not harden, form gums, or otherwise build up objectionable deposits to any substantial degree. They thus provide a durable and effective lubricant film which resists evaporation at the temperatures involved.

It may be noted that high molecular weight polymers, such as acryloids, have been suggested in the past as additives for steam cylinder oils, as in Zimmer and Morway Patent No. 2,330,773. In such cases, however, it was still necessary to employ relatively large amounts of tallow in many cases and furthermore the products seem to have lacked the superior qualities of the high grade essentially paraffinic steam cylinder oils demanded by the trade. On the basis of extensive service tests, the products of this invention are fully equal and in some respects appear to be superior to the straight paraffinic or Pennsylvania stock cylinder lubricants.

Conventional additives may be used, such as anti-oxidants, rust inhibitors, metal deactivators, viscosity index improvers, and the like, where special circumstances make such uses desirable, without departing from the spirit of the invention.

45 What is claimed is:

An emulsible, soap-free steam cylinder oil composition consisting essentially of about 87% by weight of predominantly Mid-Continent mineral lubricating oil of about 135 to 300 S. S. U. viscosity at 210° F., about 10% of a resinous propane precipitated Pennsylvania type paraffinic petroleum oil residue of substantially higher viscosity, and about 3% of tallow.

55 JONES I. WASSON.

**REFERENCES CITED**

The following references are of record in the file of this patent:

**UNITED STATES PATENTS**

| Number    | Name           | Date          |
|-----------|----------------|---------------|
| 1,924,211 | MacLaren ----- | Aug. 29, 1933 |
| 2,139,668 | Breth -----    | Dec. 13, 1938 |
| 2,298,855 | Wright -----   | Oct. 13, 1942 |
| 2,316,347 | MacLaren ----- | Apr. 13, 1943 |
| 2,339,898 | White -----    | Jan. 25, 1944 |
| 2,373,733 | Adams -----    | Apr. 17, 1945 |